

## [54] RUST REMOVAL PROCESS

[75] Inventor: Eugene S. Barabas, Watchung, N.J.

[73] Assignee: GAF Corporation, New York, N.Y.

[21] Appl. No.: 454,127

[22] Filed: Dec. 29, 1982

## [56]

## References Cited

## U.S. PATENT DOCUMENTS

|           |         |                    |           |
|-----------|---------|--------------------|-----------|
| 3,277,008 | 10/1966 | Heit               | 252/82    |
| 3,696,498 | 10/1972 | Leontaritis et al. | 427/156   |
| 3,922,394 | 11/1975 | Lozier             | 427/388.4 |
| 4,200,671 | 4/1980  | Krajewski et al.   | 134/4     |
| 4,325,744 | 4/1982  | Panayappan et al.  | 134/4     |
| 4,351,673 | 9/1982  | Lawson             | 134/3     |

*Primary Examiner*—Sadie L. Childs*Attorney, Agent, or Firm*—Joshua J. Ward; J. Gary Mohr

## [57]

## ABSTRACT

Rust is removed from metal surfaces by applying a coating of an aqueous solution of a copolymer of maleic acid and monomer of the formula  $\text{CH}_2=\text{CHR}$  wherein R represents H,  $\text{CH}_3$ ,  $\text{OR}^1$  or  $\text{OCOR}^1$  and  $\text{R}^1$  represents  $\text{CH}_3$  or  $\text{CH}_2\text{CH}_3$ . The rust becomes incorporated into the coating during drying and the coating detaches itself from the metal surface for easy removal.

10 Claims, No Drawings

## Related U.S. Application Data

- [63] Continuation-in-part of Ser. No. 364,000, Mar. 31, 1982, Pat. No. 4,424,079.
- [51] Int. Cl.<sup>3</sup> ..... B08B 7/00
- [52] U.S. Cl. ..... 134/4; 134/22.11; 252/82; 427/444
- [58] Field of Search ..... 427/309, 388.2, 327, 427/388.1, 388.4, 444, 156; 252/82; 134/3, 4, 42, 22.11

## RUST REMOVAL PROCESS

## RELATED APPLICATION

This is a continuation in part of my copending application Ser. No. 364,000 filed Mar. 31, 1982, now U.S. Pat. No. 4,424,079.

## FIELD OF THE INVENTION

The invention relates to removal of rust from metal surfaces. 10

## BACKGROUND OF THE INVENTION

Adequate removal of rust from metal surfaces in preparation for the application of paint or other protective coatings is a long standing problem. Mechanical cleaning techniques such as sand blasting, wire brush scrubbing, etc. are messy and time consuming. Previous attempts to chemically clean rusty surfaces have not been entirely satisfactory.

One particularly difficult type of metal surface to clean is the irregular surfaces found on ships, i.e., high-temperature valves, pipes, and the like. Frequently, the only cleaning method feasible is the lengthy and tiresome process of wire brushing the surface to be cleaned and then subsequently applying a solution of a wetting agent mixed with a cleaning agent to the metal surface. Such a technique suffers from the difficulty of keeping the cleaning fluid in contact with the surface to be cleaned, such as overhead objects, as well as the subsequent disposal of liquid wastes. Additionally, these solutions are often toxic, non-economical, and require large volumes of water for washing purposes.

Previous attempts to chemically remove rust have involved the use of chemicals such as inhibited hydrochloric acid, ethylenediaminetetraacetic acid (EDTA), EDTA/citric acid, etc. More recently it has been suggested that a paste of water-soluble polymer such as polyvinylpyrrolidone (PVP) and a chelating agent such as EDTA be coated onto a rusty metal surface to be cleaned. After application the paste is said to harden into a thick crust which encapsulates the rust and may be peeled from the cleaned surface and disposed of as solid waste. This process is more fully described in U.S. Pat. No. 4,325,744.

## SUMMARY OF THE INVENTION

The invention is a process for removing rust from a rusty metal surface which comprises:

- (a) applying to said rusty surface a layer of rust removal coating composition consisting essentially of an aqueous solution of a copolymer of maleic acid and monomer of the formula  $\text{CH}_2=\text{CHR}$  wherein R represents H,  $\text{CH}_3$ ,  $\text{OR}^1$  or  $\text{OCOR}^1$  and  $\text{R}^1$  represents  $\text{CH}_3$  or  $\text{CH}_2\text{CH}_3$ ; and
- (b) allowing said layer of coating composition to dry whereby rust becomes incorporated into said layer and the layer containing the rust detaches itself from the surface.

## DETAILED DESCRIPTION OF THE INVENTION

Maleic acid copolymer used in the invention may be formed by hydrolysis of precursor copolymer of maleic anhydride and monomer of the formula  $\text{CH}_2=\text{CHR}$  wherein R represents H,  $\text{CH}_3$ ,  $\text{OR}^1$  or  $\text{OCOR}^1$  and  $\text{R}^1$  represents  $\text{CH}_3$  or  $\text{CH}_2\text{CH}_3$ . The precursor copolymer may be obtained by any of the conventional methods

known for making such copolymers as exemplified for instance in U.S. Pat. Nos. 3,553,183, 3,794,622 and 3,933,763 the disclosures of which are incorporated herein by reference. In practicing the invention the

5 copolymer is used in the form of an aqueous solution generally containing between about 5 and about 60 weight percent (wt %) polymer and between about 40 and about 95 wt % water. The molecular weight of the maleic acid copolymer used may vary widely. Copolymers having K values between about 20 and about 120 or even higher are for instance generally considered suitable for use in practicing the invention.

It will be appreciated that viscosities obtainable within the preferred limits of water content and K value mentioned above may vary widely, the major variable being the amount of water used. The choice of preferred viscosity for the rust removal coating compositions of the invention will depend largely upon the intended use. For instance for lightly rusted metal surfaces it may be desired to have a thin liquid coating having a viscosity for instance between about 50 and about 50,000 centipoises (cps) such that the coating can be applied with an ordinary paint brush to a thickness between about 0.01 and about 5 mm. For many applications a relatively high viscosity, paste like coating having a viscosity e.g. between about 10,000 and about 250,000 cps may be desired. Such high viscosity coatings may be easily applied even to overhead surfaces e.g. with a putty knife to form coatings of between about 0.5 and about 20 mm or thicker as desired. The paste like form of the copolymer is especially preferable for application to vertical or overhead surfaces where excessive dripping and flowing of the coating after it is applied to the rusted surface would be undesirable.

If desired the viscosity of coating composition for use in the invention may be increased by including in the composition one or more thickening agents in an amount sufficient to increase the viscosity of the composition to the desired value. For this purpose any conventional thickening agents may be used. When used, thickening agents are frequently used in amounts between about 0.1 and about 10 wt % based on total composition. Suitable thickening agents include for instance: natural or synthetic gums such as xanthan, guar, tragacanth, etc.; cellulose derivatives such as hydroxyethyl cellulose; hydrogels such as crosslinked polymers of acrylic acid; and other synthetic thickening agents such as crosslinked poly(methyl vinyl ether/maleic anhydride). Crosslinked interpolymers of the type described in U.S. Pat. No. 3,448,088, the disclosure of which is incorporated herein by reference, are for instance suitable for this purpose.

The precursors of the copolymers for use in the process of the invention are maleic anhydride copolymers of the formula



As mentioned the copolymer is used in the form of an aqueous solution. The copolymer as used in the aqueous solution is hydrolyzed and has the general formula



lysis. The polymer solution was analyzed with the following results:

Solids: 34.97%

K-Value: 38.1

Acid Number: 210.28

Brookfield Viscosity: 3450 cps

Relative Viscosity (1%): 1.3832.

A 28 gauge sheet of black iron, the surface of which was covered with rust, was placed flat on a bench and was coated with a 1.27 mm thick 63 mm wide layer of the copolymer solution using a doctor knife.

The coated metal was allowed to stand overnight. Next morning the brittle film was found to be separated completely from the metal substrate with the rust firmly embedded in the separated film. The surface of the metal was completely free of rust.

#### EXAMPLE 4

The procedure of example 1 may be used to practice the invention using poly(ethylvinylether-co-maleic anhydride) or poly(propylvinylether-co-maleic anhydride) as the precursor copolymer rather than the poly(methylvinylether-co-maleic anhydride) of example 1. Likewise the procedures of example 3 may be followed using vinyl propionate rather than the vinyl acetate of example 3.

While the invention has been described above with respect to preferred embodiments thereof, it will be understood by those skilled in the art that various changes and modifications may be made without departing from the spirit or scope of the invention.

What is claimed is:

1. Process for removing rust from a rusty metal surface which comprises:

(a) applying to said rusty surface a layer of rust removal coating composition consisting essentially of an aqueous solution of a copolymer of maleic acid and monomer of the formula  $\text{CH}_2=\text{CHR}$  wherein R represents H,  $\text{CH}_3$ ,  $\text{OCOR}^1$  and  $\text{R}^1$  represents  $\text{CH}_3$  or  $\text{CH}_2\text{CH}_3$ ; and

6  
(b) allowing said layer of coating composition to dry whereby rust becomes incorporated into said layer and the layer containing the rust detaches itself from the surface.

5 2. Process according to claim 1 wherein the coating composition contains between about 5 and about 60 wt % copolymer and between about 40 and about 95 wt % water.

10 3. Process according to claim 1 wherein the coating composition has a viscosity between about 50 and about 250,000 cps.

15 4. Process according to claim 2 wherein the coating composition is applied to the rusty surface in a layer between about 0.01 and about 20 mm thick.

5. Process according to claim 4 wherein the layer of applied coating composition is allowed to dry for between about 0.5 and about 8 hours.

6. Process according to claim 1 wherein:

(a) the coating composition consists essentially of between about 5 and about 60 wt % of said copolymer and between about 40 and about 95 wt % water;

(b) the coating composition is applied to the rusty surface to form a layer between about 0.01 and about 20 mm thick;

(c) the coating composition has a viscosity between about 50 and about 250,000 cps; and

(d) the applied coating composition is allowed to dry for between about 0.5 and about 8 hours whereby the rust becomes incorporated into the layer of coating composition and the layer becomes detached from the metal surface.

7. Process according to claim 1 wherein R represents hydrogen.

35 8. Process according to claim 1 wherein R represents  $\text{CH}_3$ .

9. Process according to claim 1 wherein R represents  $\text{OCOR}^1$  and  $\text{R}^1$  represents  $\text{CH}_3$ .

10. Process according to claim 1 wherein R represents  $\text{OCOR}^1$  and  $\text{R}^1$  represents  $\text{CH}_2\text{CH}_3$ .

\* \* \* \* \*